

Patented July 26, 1949

2,477,244

# UNITED STATES PATENT OFFICE

2,477,244

## STABILIZED ORGANIC SULFUR-CONTAINING COMPOSITION AND METHOD OF PREPARING SAME

James W. Gaynor, Hammond, Ind., assignor to Standard Oil Company, Chicago, Ill., a corporation of Indiana

No Drawing. Application June 26, 1946,  
Serial No. 679,593

6 Claims. (Cl. 252—48.2)

1

This invention relates to an improved method of inhibiting the evolution of hydrogen sulfide from organic sulfur-containing compounds from which hydrogen sulfide is normally evolved, and to organic sulfur-containing compositions stabilized against hydrogen sulfide evolution.

Many organic sulfur-containing compounds evolve hydrogen sulfide in the course of their normal use or in storage. Because of the obnoxious odor of hydrogen sulfide gas the evolution of hydrogen sulfide from such organic compounds is very objectionable. Examples of such organic compounds are sulfurized terpenes, sulfurized olefins and olefin polymers, sulfurized fatty oils of animal and vegetable origin, sulfurized sperm oil, sulfurized mineral oils and the like. Not only is the use of such organic compounds restricted because of the obnoxious odor of the evolved hydrogen sulfide, but the use of compositions containing various amounts of such organic sulfur compounds is often restricted because of this nuisance. For example, lubricants such as hydrocarbon lubricating oils frequently contain sulfurized materials to impart thereto various desired properties such as extreme pressure properties, anticorrosion properties and the like. However, such lubricants during service or in storage evolve hydrogen sulfide which is found highly objectionable by the users of such lubricants.

It is, therefore, an object of the present invention to provide an improved method of inhibiting the evolution of hydrogen sulfide from organic sulfur-containing compounds which normally evolve hydrogen sulfide during service or storage. Another object of the present invention is to provide a method whereby organic sulfur-containing compounds which evolve an obnoxious hydrogen sulfide odor are rendered inoffensive. Another object of the invention is to provide organic sulfur-containing compositions stabilized against hydrogen sulfide evolution. Other objects and advantages of the invention will become apparent from the following description thereof.

I have discovered that the evolution of hydrogen sulfide from organic sulfur-containing compounds can be substantially inhibited by adding to such compounds an alpha-beta unsaturated ketone in small but sufficient quantities to substantially inhibit the evolution of hydrogen sulfide; suitably in concentrations of from about 0.001% to about 25.0%, and preferably from about 0.01% to about 5.0% by weight based upon the sulfur-containing compounds. The alpha-beta unsaturated ketone may be an alpha-beta unsaturated aliphatic, cycloaliphatic or aromatic ketone.

By an alpha-beta unsaturated ketone as used herein and in the appended claims is meant a ketone containing at least one ethylene linkage

attached to the carbonyl group, as represented by the structural group



Operable unsaturated ketones include those having one or two double bonds conjugated with the carbonyl group. The ketone group and/or the double bond may also be present in a cycloaliphatic ring.

The following specific compounds are representative of alpha-beta unsaturated ketones:



Phorone



Mesityl oxide



Benzal acetone



Dibenzal acetone



Difurfural acetone



Isophorone



Butylidene acetone



Methyl vinyl ketone



Coumarin



Benzal acetophenone

The aromatic nuclei in the alpha-beta unsaturated ketones may be alkylated or contain other substituents, such as, for example hydroxyl, amino and nitro groups.

While the foregoing compounds are all effective in inhibiting the evolution of hydrogen sulfide from organic sulfur-containing compounds, it is not to be implied that all are equivalents, since their specific activity varies to some extent.

The effectiveness of the alpha-beta unsaturated ketones in inhibiting the evolution of hydrogen sulfide from organic sulfur-containing compounds is illustrated by the following tabulated data. These data were obtained by diluting a composition containing an organic sulfur-containing compound with an SAE 10 motor oil, placing the mixture in a container, and maintaining the mixture therein at a temperature of 200° F. while passing nitrogen through the mixture at a rate of one liter per hour. Preformed hydrogen sulfide was first removed by passing nitrogen through the mixture for one-half hour. The exit tube from the container was then connected to two vessels in series and containing lead acetate solution, the first of which had a known volume and concentration. The time required for 100 grams of the test material to evolve 9 milligrams hydrogen sulfide was noted by the formation of PbS in the second vessel. The control was a mineral lubricating oil additive composition containing a KOH neutralized product of P<sub>2</sub>S<sub>5</sub> and an isobutylene polymer, a sulfurized mineral oil and a sulfurized terpene.

| Sample               | Hours for 100 grams of Sample to Evolve 9 mg. Hydrogen Sulfide |
|----------------------|----------------------------------------------------------------|
| Control              | 0.50                                                           |
| Control+0.5% phorone | 3.65                                                           |
| Control+1.0% phorone | 9.10                                                           |
| Control+2.0% phorone | 25.0+                                                          |

The above data show the stabilizing effect of alpha-beta unsaturated ketones on the evolution of hydrogen sulfide from organic sulfur-containing materials. While these data were obtained with a specific lubricant composition using a particular oil-soluble detergent, namely a KOH neutralized reaction product of P<sub>2</sub>S<sub>5</sub> and an isobutylene polymer, and particular organic sulfur-containing compounds, namely a sulfurized mineral oil and a sulfurized terpene, other oil-soluble detergent-type additives and other organic-sulfur-containing materials can be used. For example, the oil-soluble detergent additive may be a neutralized reaction product of a phosphorus sulfide and a hydrocarbon as described in U. S. 2,316,082.

Many lubricant compositions contain from about 0.01% to about 10% by weight of an oil-soluble detergent-type additive and an organic sulfur-containing additive, the former to impart varnish inhibiting or removing properties to the lubricant, and the latter to impart lubricating and/or corrosion inhibiting properties. The oil-soluble detergent-type additive is frequently responsible for an increased rate of hydrogen sulfide evolution from the organic sulfur-containing additive. Under these conditions the addition of the herein-disclosed alpha-beta unsaturated ketones effectively inhibits the evolution of hydrogen sulfide from such compositions.

The term "oil-soluble detergent-type additive"

as used herein and in the appended claims means an organic compound having the property of substantially inhibiting the formation of varnish in internal combustion engines and/or the property of removing varnish formed in such engines.

While I have described my invention by reference to specific embodiments thereof, these have been by way of illustration, and the invention is not to be limited thereby, but includes within its scope such modifications as come within the spirit of the appended claims.

I claim:

1. A lubricant composition comprising a major proportion of a hydrocarbon oil and an organic sulfur-containing compound which normally evolves hydrogen sulfide and from about 0.001% to about 25% by weight based upon the sulfur-containing compound of an alpha-beta unsaturated aliphatic ketone.

2. A lubricant composition as defined in claim 1 in which the alpha beta unsaturated aliphatic ketone is phorone.

3. A lubricant composition consisting essentially of a major proportion of a hydrocarbon oil, an oil-soluble detergent type additive consisting essentially of a neutralized reaction product of a phosphorus sulfide and a hydrocarbon, an organic sulfur-containing compound, which normally evolves hydrogen sulfide, and from about 0.001% to about 25% by weight, based upon the sulfur-containing compound, of an alpha beta unsaturated aliphatic ketone.

4. The method of inhibiting the evolution of hydrogen sulfide from an organic sulfur-containing compound which evolves hydrogen sulfide comprising adding to said compound from about 0.001% to about 25% by weight, based upon the sulfur-containing compound of an alpha-beta unsaturated aliphatic ketone to substantially inhibit the evolution of hydrogen sulfide from said organic sulfur-containing compound.

5. The method of claim 4 in which the ketone is phorone.

6. The method of inhibiting the evolution of hydrogen sulfide from a lubricant composition containing a major proportion of a hydrocarbon oil and a sulfurized organic compound which normally evolves hydrogen sulfide comprising employing with said lubricant composition from about 0.001% to about 25% by weight based upon the sulfur-containing compound of an alpha-beta unsaturated aliphatic ketone.

JAMES W. GAYNOR.

#### REFERENCES CITED

The following references are of record in the file of this patent:

#### UNITED STATES PATENTS

| Number    | Name    | Date           |
|-----------|---------|----------------|
| 2,130,080 | Evans   | Sept. 13, 1938 |
| 2,158,724 | Kilgore | May 16, 1939   |
| 2,367,344 | Evans   | Jan. 16, 1945  |

#### OTHER REFERENCES

Fieser and Fieser, *Organic Chemistry*, D. C. Heath & Co., Boston, 1944, page 725.

Houben, "Die Methoden der Organischen Chemie," vol. II, 3d edition, page 1008.